

April 14, 1931.

M. E. EVANS

1,800,249

## METAL CASTING PROCESS AND APPARATUS

Filed July 25, 1929

3 Sheets-Sheet 1



FIG. 6.

INVENTOR  
*Martin E. Evans.*

April 14, 1931.

M. E. EVANS

1,800,249

## METAL CASTING PROCESS AND APPARATUS

Filed July 25, 1929 3 Sheets-Sheet 2



107 FIG. 3



FIG. 6

FIG. 5



FIG. 8



FIG. 7

**INVENTOR**

Martin Evans

April 14, 1931.

M. E. EVANS

1,800,249

## METAL CASTING PROCESS AND APPARATUS

Filed July 25, 1929 3 Sheets-Sheet 3



FIG. 10



INVENTOR  
*Martin E. Evans.*

## UNITED STATES PATENT OFFICE

MARTIN E. EVANS, OF KANKAKEE, ILLINOIS

## METAL-CASTING PROCESS AND APPARATUS

Application filed July 25, 1929. Serial No. 380,963.

The invention relates to the art of metal casting and particularly to means and methods for casting refractory metals and alloys into bodies of a wide range of sizes, shapes, 5 and mechanical mixtures. Masses of metal as large as steel ingots and as small as steel rods are contemplated to be produced by this invention which has for one object the production of metal bodies free from piping, 10 blow holes, segregation, large crystals and internal stresses that usually are associated with metal casting.

Another object of the invention is the production of castings of composite metals of 15 different melting temperatures.

Another object of the invention is the production of castings of composite metals so that each metal retains the physical properties in the casting that it would have if cast 20 separately.

Another object is to produce metal castings of fibrous structure.

Another object is to produce a metal casting continuously.

25 Another object is to produce a metal casting at a rate uncontrolled by the usual cooling rate of the metal cast.

Another object is to produce castings that solidify from the body center towards the 30 periphery instead of in the reverse order which is usual.

Another object is to provide a washing and purification of the metal as it is being cast.

Another object is to reduce the nonmetallic 35 inclusions of metals cast.

Another object is the placement of metallic particles in definite relative positions in a casting.

Another object is to provide a means for 40 maintaining a welding heat in the portions of a casting already cast pending the placement thereon of successive portions, that are plastic and at a welding heat.

Another object of the invention is the production of a casting with a homogeneous mixture of metals of widely varying specific 45 gravity and melting points.

To these ends special processes and means for carrying them out are provided which 50 will be readily understood from the follow-

ing remarks and descriptions and accompanying illustrations.

In the usual art of casting metals, various difficulties are encountered which cause defects in the cast product varying with the 55 quantity of metal involved in the casting operation.

Considering the casting of steel as an example, and particularly large ingots, piping, blowholes, segregation, large crystals and internal stresses are physical conditions that are more or less present collectively in spite of various expedients employed to obviate them. They are all the result of the phenomena accompanying the cooling of a large 60 mass of metal from the liquid to the solid state. To obviate them the present invention contemplates the cooling of small particles of molten metal to the plastic or weldable 65 state and successively welding them together 70 in the order of their cooling.

Because of a premature chilling and solidifying of smaller masses of metal when subjected to the cooling action of molds or apparatus contacting with the metal, the production of strips or small castings of steel have been difficult. To obviate this difficulty, the 75 present invention provides a heat conveyor or vehicle and a temperature regulator in the form of a slag of characteristics compatible 80 with the character of the metal with which it cooperates. The same heat conveyor and temperature regulator is employed in the production of the larger mass of metal, which is comparable to the usual standard ingot, as is used 85 for the production of strips or small castings.

When two pieces of steel are to be welded together it is customary to coat them with a flux or welding cinder, then to heat them to a welding temperature and to hammer them together at the point of welding temperature thereby forcing the welding cinder aside and effecting a chemical union of the metal. A portion of the welding cinder is inevitably 90 entrapped between the two pieces but not in quantity sufficient to be detrimental. Continued hammering during the cooling of the weld prevents crystal growth and preserves the quality of the metal. The welding cinder 95 serves the very useful purpose of protecting 100

the metal from oxidation during the operation. The present invention contemplates the constant repetition of these operations with particles of metal as they are changed from the molten to the plastic or welding state. Pressure between the weldable particles is quickly applied after the particles attain the weldable state, particle adhering to particle as a result thereof and the excess welding cinder or slag being expressed piece-meal therefrom. The gradual accumulation of particles results in the building up of a solid metal body including a minimum of the fluxing or welding cinder by reason of the particle by particle welding and expressing operations.

It is a coincidence that the welding cinder or flux most suitable for the practice of this invention in casting steel is the siliceous slag used in the hand puddling of wrought iron which is in reality in its final stages a welding operation. However, the product resulting from the practice of the present invention is markedly different from the product generally known as wrought iron wherein the welded mass attains considerable size before it is subjected to pressure to remove the slag content or reduce it. This means that particles of welded metal must be forced apart to provide a path of exit for the slag, the path being subsequently welded shut. Enormous pressures necessitating expensive apparatus are required for these operations and in proportion to the masses of material involved in the squeezing and welding operations. Hand puddling operations involve masses of fifty to two hundred pounds of metal. Mechanical puddling operations or mechanical production of wrought iron involve masses up to two thousand pounds of metal. It is at once apparent that these masses must include considerable slag inclusions and representative samples show 2% to 5% inclusions after squeezing.

In the practice of the present invention, in some cases squeezing and pressure are exerted as the particles of metal are changed from the molten to the crystal or plastic state and not as a separate and subsequent operation as in the before-mentioned methods of wrought iron production, the product having a variable slag content down to less than one and one-half per cent. The slag serves as a vehicle in which the metal is conveyed while changing from a molten or fluid condition into a plastic or crystal state and delivered in close proximity to a body of worked metal in a condition for receiving further additions by welding. The continued arrival of slag particles with the metal particles conveys heat to and regulates the temperature of the growing or accumulating body of metal, since heat is continuously being abstracted from the accumulating body of metal by conduction and radiation. The energy of the moving

particles of both slag and metal is utilized to effect the initial union between metal particles, making welding operations successful at somewhat lower temperatures than are employed in puddling and mechanical wrought iron production and at the same time expressing portions of slag from between metal particles and effecting a welding action in the vicinity of the displaced slag. However, simple flow of cast metal and contact of successive particles also is contemplated to build the body of cast metal and its associated material.

This invention makes available for the first time mechanical mixtures of metals which if mixed together in the molten state for casting dilute and intermix to form a uniform

analysis. Thus, a high carbon steel and a low carbon steel when brought together in molten states in equal quantities blend together to produce a medium carbon steel of uniform analysis.

However, by the present invention particles of steel of each carbon analysis are crystallized and brought together in the state admitting of welding and

like particles are successively brought together in a regular manner whereby a mass of the two kinds of steel in regular alternation is accumulated while retaining a portion of their casting heat.

As an instance of the practical application of such a steel we may refer to rope wire steel. Ordinarily such

steel varies from .50 per cent carbon with a tensile strength of 180,000 lbs. per square inch to .80 per cent carbon with a tensile

strength of 265,000 lbs. per square inch after heat treatment in wire form.

If mixed together in equal quantities the resulting molten steel would have approximately .65 carbon with physical characteristics intermediate

those of the original metals. By reducing particles of each steel separately to a crystal,

plastic or welding condition and placing them one upon the other in regular alternation an accumulation of uniformly mixed metals re-

sults, the one of .50 carbon having its usual strength, pliability and ease of bending and the other of .80 carbon having its usual high strength, relative stiffness and low elongation.

However, because of the fibrous nature of the mixture, the relatively small cross sec-

tion of each metal particle, and the variable metallic makeup, improved resistance to

bending, vibration, twist and shock are obtained.

Instead of mixing metals of the same base different metals may be advantageously com-

bined. Copper wire used as long span elec-

trical conductors lacks sufficient strength and is usually reinforced by steel in the form of

separate wire. By the practice of the present

invention the steel is reduced in a suitable

slag to a plastic state and the copper likewise

conditioned from either a comminuted or a

molten state and in the relative metallic pro-

70

75

80

85

90

95

100

105

110

115

120

125

130

135

140

copper they are assembled in alternation in the before-mentioned proportions, the copper completely enclosing the steel. The accumulated mass of copper and steel when worked down into wire possesses the conductivity of the copper in the desired degree and the combined strength of the copper and steel sufficient for requirements. It is obvious that varying proportions of metals may be so accumulated, the proportion just mentioned being by way of example only.

These examples illustrate the procedure by which various metal combinations may be selected and accumulated. Small slag inclusions, inevitably entrapped with the metal or metals in any given accumulation of metal contribute a fibrous structure to the mass as the further working of the metal proceeds. Because of the relatively small aggregate of slag in any one position and the regularity of the positioning among the metal particles, a uniformity and degree of fineness of fibre is obtained which gives the metal marked superior qualities that enable it to resist vibration and shock. Fatigue of the metal is confined to individual fibres which when they break in two because of their individual character do not spread a crack across adjacent fibers whereas a crack on the surface of ordinary metal subjected to vibration travels continuously across the body until it is severed.

By a suitable arrangement of the mechanism employed in the operations of assembling metal particles after the manner of this invention, the casting or assembling operation is made continuous. To this end, a continuous slag supply, a continuous metal supply, a continuous slag departure and a continuous metal departure are arranged while a continuous separation of slag and metal is effected as the metal particles are sequentially welded together. The arrangement maintains the growing or accumulating end of the metal mass at a welding temperature so that arriving metal particles have no difficulty in effecting contact and substantial union under either flow or pressure with their sequential forerunning like particles.

The continuous casting arrangement is free from the usual limitations imposed by the cooling rate of the metal by reason of the heat supplied by the slag. Heretofore, failure of continuous casting has been caused by lack of means to regulate the heat of the last cast particle to accommodate union with the next contacting particle. In the present invention the heat supplied by the slag as it dissipates from the metal may be replaced by heat from more slag whereas the usual casting method is solely dependent upon utilizing the heat of the cast metal.

The first sectional portion of the continuously produced metal may be manipulated in a variety of ways whereby its size is in-

creased. Successive additions of metal may be made on both sides as the operation of casting continues from the molten state. Also the section of the metal may be immersed in molten slag at a welding temperature and folded upon itself as it grows in length with each fold pressed upon the preceding one expressing the slag from therebetween and effecting a welded union of adjacent surfaces. The folding operation may be continued until a body of metal accumulates of dimensions in accord with those of steel ingots in ordinary production. Because of the method of assembly of the metal particles the cooling of the particles has taken place in the sequence of their placement resulting in the large mass of metal being free from the piping and other associated defects.

The successive layers of welded and squeezed metal may be produced directly in a bath of slag. In this practice a layer of metal particles is provided over the area of the bath and subjected to pressure effecting welding and expression of slag from among the metal particles, successive layers being produced in like manner to build up a homogeneous mass with a minimum of slag inclusions.

In the practice of the invention, the contact of slag and metal results in the washing of the metal and the release of occluded gases so that the metal as solidified and finally assembled has a so-called homogeneous and fibrous characteristic condition when the slag used is in excess of that to be entrained in the metal to produce wrought iron. The washing operation of the slag on the metal produces a cleansing effect which is highly advantageous in the manipulation of ferrous metals particularly. Due allowance for removal of elements by the excess slag is taken by providing an excess of such elements in the molten body of metal to be cast so that the analysis of the final metal body will accord with specification requirements.

In the practice of this invention in the art of casting of single metals continuity of contact of the metal particles in their molten state and in the subsequent plastic and welded states is maintained. Disintegration of the metal and intermingling of slag and metal particles are not desired for the reason that a higher percentage of slag would inevitably be entrapped and thus alter the character of the product desired. A continuous stream of metal or a continuous sheet of metal in the molten or plastic condition are desired with which or through which slag particles pass at a temperature which produces or maintains a plastic or welding condition of the metal. The purpose is to secure the quick crystal formation or solidification of the metal to avoid defects which ordinary expedients in casting do not obviate and to refine the metal structure by working. The

quantity of slag involved must necessarily be greater than the quantity of metal in the operations involving washing ferrous metals in order to preserve the continuity of the operations where the slag is flowing and the movement of the metal after reduction to welding heat is relatively slow. The change in the rate of flow or linear movement of the metal and the change in direction of flow of the slag converts the energy of movement into force effective to force slag through the metal and to weld together newly associated metal particles under some conditions of operation.

15 The stream or sheet of molten metal provided in the casting operation under consideration acquires an increasing momentum as it departs from its point of origin thereby becoming extremely attenuated. As the 20 attenuation longitudinally increases the particles are crowded together in a cross sectional direction thereby providing metal for maintaining continuity. When a sufficient body of metal is provided the attenuation 25 may be effected in the cross sectional direction also. Crystallization of the metal and its accumulation may occur at a variety of points in the path provided and means for removal of the accumulations are provided 30 and used in accordance with the quantity and condition of the metal.

In casting a mixture of metals, the continuity of the low percentage metal in the mixture while in the molten condition necessarily must be broken though it may again be established in the mixed body of metal.

Various means for effecting the gradual accumulation of metal particles from a molten state into a mass of metal free from 40 physical defects are illustrated and described, the means chosen for any particular application being chosen for its special adaptability to the size of metal accumulation desired and to the characteristics of the metal mixture to 45 be accumulated.

Referring to the drawings,

Fig. 1 shows a side and sectional view of a centrifugal casting machine.

Fig. 2 shows a side view of the centrifugal 50 casting machine at right angles to the view of Fig. 1.

Fig. 3 shows a sectional view of a modification of the rotor illustrated in Fig. 1.

Fig. 4 shows a plan view of the rotor in 55 Fig. 3.

Fig. 5 shows the relative directions of movement of centrifugally cast material and the wall upon which it is cast.

Fig. 6 shows another view of the movement of centrifugally cast material as it is deposited on a receiver.

Fig. 7 shows a rotary deflector and anvil on which rests an accumulation of metal.

Fig. 8 shows a casting and coating operation in progress between rolls.

Fig. 9 shows an accumulation of compressed cast metal.

Fig. 10 shows a side view of a roll type casting machine.

Fig. 11 shows a sectional view along line 70 A—A at right angles to the view of Fig. 11.

Fig. 12 shows a plan view of a pair of casting rolls.

Referring to Fig. 1 and Fig. 2, on a base plate 1 uprights 2, 3, 4, and 5 are mounted 75 to which is attached a mid-cross plate 6 circular in shape and split across its diameter.

A bearing 7 in the center of the mid plate carries an inner lining 8 and an upper end ball race channel 9 which supports a spindle 10. The lower end of the spindle 10 carries a spider 11 on the outer rim of which a pulley 12 is mounted with a belt 13 thereon operated and controlled from a source not shown. On the upper end of the spindle 10 a shoulder 14 carries a ball race channel 15 co-operating with the race channel 9 on the mid-cross plate to give stability to the spindle 10. The shoulder 14 also carries openings 16 into which fit extensions from a superposed bowl 17. The bowl has a depressed cup section 19 from which a wall 20 extends upwardly. At the quarter points of the bowl 17 downward exits 21, 22, 23, 24 through the cup 19 are provided. Rotary motion of the spindle 10 is transmitted to the bowl 17 through the extensions thereon fitting into the openings 16 of the spindle. In the hollow of the spindle 10 frictionless bearings 26 and 27 support a slidable shaft 30 fitted with sliding keys 28 and 29 operative in the frictionless bearings 26 and 27. The upper end of the slidable shaft 30 extends through and opening 31 in the base of the bowl 17 and fits into the base opening 32 of a rotary anvil 33 and deflector 34. Below the spindle 10 and adjacent the pulley 12 thereon a pulley 35 carrying a belt 36 is mounted on the slidable shaft 30 and transmits motion thereto from a source not shown.

The lower end of the slidable shaft 30 is supported by a shoulder 37 thereon on a frictionless bearing 38 which receives an up and down motion through the rotation of a nut 39 contacting therewith. The lower end of the slidable shaft 30 extends through the nut 39 and into an associated threaded stationary base stud 40 resting on and attached to the base plate 1. A yoke 41 carrying a worm 42 encloses the nut 39 and positions the worm for engagement with a worm-threaded shoulder 43 on the nut so that rotation of the worm causes rotation of the nut on the threaded stud which gives a longitudinal movement to the shaft 30 and to the anvil 33 and deflector 34 thereon. Motion is transmitted to the screw 42 by a shaft 44 and universal joints 45 and 46 thereon from a stub shaft 47 in a bearing 48 attached to a frame upright 2. The stub shaft 47

80

85

90

95

100

105

110

115

120

125

130

carries a pulley or hand wheel 49 to which power is applied when up and down motion of the anvil and deflector is desired.

Resting on the mid-cross plate 6 and between the frame uprights 2, 3, 4, and 5, is a circular chamber with an upright outer wall 50 enclosing the rotatable bowl 17 and its associated anvil 33 and deflector 34. An inwardly projecting rim 51 extends around the top of the chamber having an opening sufficiently large to accommodate the removal of the bowl 17 and associated anvil 33 and deflector 34. The bottom 52 of the circular chamber extends inwardly to a point adjacent the inner portion of the bowl at which point an inner wall 53 extends upwardly to the vicinity of the bowl 17. A refractory lining 55 fits the full inside portion of the circular chamber, a narrow opening 56 on a level with the chamber bottom 52 and of a height approximating the height of the inner wall 53 of the chamber leads to a spout 57 for draining the chamber into a conveniently placed ladle 58.

On one of the long frame uprights 2 a pair of brackets 59 and 60 support a stationary shaft 61 carrying collars 62, 63, and 64 which position three cross bars 65, 66, 67 pivotally mounted on the upright shaft 61, the opposite end of the cross bars being detachably engaged by bolts 68, 69, 70, to the long frame upright 4 opposite the brackets 59 and 60. The cross bars 65, 66, and 67, have cone shaped chambered mid sections 71, 72, 73 respectively into which fit cone shaped shells 74, 75, 76 which are concentric with the bowl 17 below them and which are positioned one above the other with a space between them such that the three shells occupy positions on an imaginary continuous enclosed cone. The end 77 of the lowermost cone is positioned in the vicinity of the point 78 of the anvil 33 with an intervening space 79 sufficiently large to accommodate the passage of liquids in their downward course from the shells 74, 75, 76. The upper edges of the shells 74, 75, 76 are curved outwardly and downwardly forming dams 81, 82, 83, respectively, and downwardly and again upwardly forming chambers 84, 85, 86 respectively with rims 87, 88, 89 respectively and with spaces 90 and 91 between the shells. The shells are sufficiently refractory to withstand the heat of the materials contacting with them in the operations involved. The rims 87, 88, 89, are sufficiently high to cause material poured into the chambers 84, 85, 86 to flow over the dams 81, 82, 83 and down the inside of shells 74, 75, 76 to the common point 78 of the anvil 33 below them. The cross bars 65, 66, 67 may be interchanged to position the shells 74, 75, 76 to accommodate different pouring requirements. The interspaces 90 and 91 between the shells provide access for hand tools used in clearing accumulations with-

in the shells during operations. Extending across the tops of the uprights 2 and 4 which support the cross bars 65, 66 and 67 is a cross bar 80 serving as a tie bar to the uprights to which it is attached and as a bearing for supporting hand bars or mechanically operated bars for clearing the inside of the shells 74, 75, 76.

Variations in the method of operation of the mechanism thus far described permit the production of a variety of products. The preferred method of operation in the casting of steel requires that into each of the chambers 84, 85, 86, of the conical shells 74, 75, 76, hot molten slag should be poured at a temperature approximating the melting point of steel and in quantity sufficient to overflow the shell dams 81, 82, 83 and the inner surfaces of the shells 74, 75, 76, from which it flows onto the rotating anvil 33 and the deflector 34 which pass it on to the rotating wall 20 of the bowl 17 from which it flows out of the openings 21, 22, 23, 24, in the cup of the bowl 17 to the chamber lining 55 around and under the bowl and out of the chamber opening 56 and the spout 57 to the slag bucket 58. After passage of the slag has heated the various parts with which it contacts to temperatures high enough for operating purposes, the slag flow is stopped.

Molten steel is then poured into the mid-positioned chamber 85 while molten slag or welding cinder at a temperature around the welding point for steel is poured into the upper positioned chamber 84, the pouring of the slag and steel at rates of two to three volumes of slag to one volume of steel causing an overflow of the dams 81 and 83 with the slag impacting upon the steel as the latter overflows its chamber dam 82. The impact of the slag on the steel accelerates the flow of the latter over the lower positioned shells 75 and 76 while an interchange of heat between the slag and steel occurs. The greater weight of the steel keeps it in contact with the refractory shell with the slag on top protecting from atmospheric oxidation. Molten slag poured into the lower positioned chamber 86 overflowing the shell dam 83 contacts with the steel and is entrained therein and forced therethrough providing a washing action on the steel. Impact of the slag and steel on the tapering anvil gives them a spreading action following the attenuation accompanying the flow down the shells. The slag on the inside of the descending tube of slag and steel is forced through the steel as the mass is deflected from its vertical path. Rotation of the deflector 34 is in one direction and of the bowl wall 20 in the opposite direction. The centrifugal action of the deflector adds momentum to the mass of slag and steel as it is impelled against the bowl wall 20. Impact of the mass on the rotating bowl wall 20

causes a spreading action, greatest in the direction of rotation of the bowl, forcing the slag from perforations in the metal and welding the metal with a minimum of slag inclusions. An up and down motion of the deflector effects a folding of the metal upon itself as it accumulates on the bowl wall 20. The up and down motion is produced by manual or other operation of the elements 10 identified by numerals 30 to 49 inclusive in the preceding paragraphs.

The excess slag passes from the bowl by a path dependent upon the rate of bowl rotation. If the rate is relatively slow, the exit 15 is by downward openings 21, 22, 23, 24, from the bowl cup and if relatively fast the exit is by the upward path over the bowl wall 20, to the chamber lining 55 and in either case out of the chamber opening 56 and over 20 the spout 57 there positioned into the slag bucket 58.

The change from the molten to the plastic state by the steel becomes operative with the first contact of slag and steel in a degree 25 dependent upon their differences in temperature and continuing until the steel is welded into position in the accumulation on the bowl wall. The volume of steel may be lessened and the volume of the slag inclusions forms 30 within the mid positioned shell and moving downwardly under the impulse of the moving slag and compressing in diameter into the lower positioned shell where it is further compressed and welded. If the taper 35 of the shells does not accommodate the movement of the ring, force thereon by hand or power tools may be exerted downwardly through the center forcing the ring past the bottom 77 of the lower shell and over the 40 anvil 33. It is obvious that as the metallic ring descends its entrained slag content decreases due to the expressing of slag toward the inside of the ring in consequence of the 45 change from the large to the smaller diameter. Successive rings deposited on the anvil 33 and continually washed by the descending slag at welding temperature weld together to form a mass of slag and steel somewhat 50 approaching puddled iron in its slag content.

Removal of the metal cast in the bowl is effected by removing the bolt 70 fastening the lower cross bar 67 to the frame upright 4 and swinging the bar about the pivot shaft 55 61 at its other end thereby removing the lower shell 76 from over the bowl 17, and then lifting the ring of metal from the tapered wall 20 of the bowl through the upper opening of the bowl chamber and sidewise 60 through the space cleared by the lower shell travel.

Removal of the metal impaled on the anvil 33 and deflector 34 is effected in a similar vertical and sidewise lifting movement.

65 Removal of metal from a shell is readily

effected upwardly while the superposed shell is swung to one side.

After the metal is removed, it is subjected to rolling or other metal working operations while still possessing some of its heat of 70 casting.

By making the intervening space 79 between the lower shell 77 and the point 78 of the anvil 33 sufficiently large, successive rings 75 of metal may be removed therethrough from the deflector 34 and the anvil 33, thus making the operation of the process practically continuous. Also by making it sufficiently small, a ring of metal may contact with both the superposed shell and the under poised 80 anvil practically closing the passage from the shell until pressure on the ring forces it downward on the anvil. With the shell sufficiently well supported, the up and down motion of the anvil may be utilized to effect 85 the working and withdrawal of the metal from the shell.

It is apparent that various reacting materials may be introduced into the metal or metal and slag through the spaces 90 and 91 between the shells or through the upper end openings of the shells so that reactions more or less violent may safely take place within the shell enclosure as the metal flows downward within the shell from the chamber around its upper section. Also the character of the slag or cooling medium may be other than that of the siliceous pudding cinder. The apparatus lends itself readily to practices such as that of Patent 511,648 100 by Parkinson using a slag not of puddling characteristics. Obviously the mixing shells 74, 75 and 76 may be used to entrain slag particles in metal without rotating the anvil 33 and the bowl 17.

A variety of metals may be poured individually each into its individual shell chamber to pursue its course downward within the shells with the other metals to the anvil and deflector from whence they may be deposited on the revolving wall 20 of the receiving bowl 17. Poured at rates that permit cooling to take place to a plastic state of at least one metal on the deflector, deposition on the revolving wall 20 may effect a 115 welding of the particles in their positions, an action which is contrary to the action where ordinary centrifugal casting is used. However, special apparatus may advantageously be employed for simultaneously casting different materials in a single body and such apparatus is now to be considered.

In Fig. 3 and Fig. 4 sectional and plan views respectively of modifications of apparatus are shown.

Cooling tanks 93, 94, 95 are disposed at quarter points between the frame uprights 2, 3, 4, 5 over hooks 97, 98, 99 respectively and retained in position thereon on the outer wall 50 of the large operating chamber. 120

Pipes 101, 102, 103 on the respective tanks furnish passages for the suitable cooling medium. Inside the large chamber and at the quarter points opposite the frame up rights 2, 3, 4, 5, are positioned the dividers 104, 105, 106, 107, which are operative to divide the metal deposited on the inside of wall 50 into lengths facilitating their removal. The bowl 17 is provided with an inner lower ring 108 held in position by frictional engagement, and inner upper ring 109 held in position by clips 110 extending through passages 111 in the rim 20 of the bowl 17. Rotation of the bowl causes the clips 15 to retain their position by centrifugal action. The position of the usual anvil 33 and deflector 34 is occupied by a special distributor 112 adapted to rotary movement through engagement with the slideable shaft 30. Concentric chambers 113 and 114 have separate exit passages 115 and 116 respectively extending radially and opposite from each other. The exit passages are of a converging channel shape so that a continuous stream of metal may be supplied to the ori- 25 fices 117 and 118 as the rate of travel in the passages increases during rotation. An accessory deflector plate 119 on the upper side of the rotor serves during rotation to direct any material dropped thereon into the surrounding bowl 17 or into the large chamber beyond the bowl in the event that the bowl is not in its operating position. The concentric position of the chambers 113 and 114 30 with respect to the superposed pouring shells is contemplated in order that each chamber may be supplied with material in accordance with a chosen operating plan.

In operation, the special modification just described may advantageously be used for the production of the special rope wire steel previously referred to; steel of the higher carbon grade and slag may be poured in the center chamber 113 and steel of the lower carbon grade and slag into the outer chamber 114 at rates and temperatures so that as each steel emerges from its nozzle a plastic condition or near plastic condition is present as the centrifugal action carries the metal to bowl lining 122 for spreading therein. When the metal arrives in a stream, any given particle of metal must make half a revolution relative to the stream source when the two streams are operative before another particle of different metal is spread thereon giving a time interval and means for cooling from plastic to welded state, and the impact of the next particle provides the necessary force to complete the welding operation of the preceding superposed particles. Thus in effect a thin strip of metal and cinder is deposited upon which a succeeding layer is placed, the two layers cooling to welding temperatures and succeeding layers by impact thereon completing the welding opera- 55

tion. The continuity of the operation builds up a body of composite metal and cinder of a fibrous structure new to the art.

The structure of the casting has a smaller grain structure than is found in bodies of metal of the same size cast by previous methods for the reason that the time interval between pouring and solidification of any given particle is less in the practice of the present invention and the solidification takes place in progression from one side of the casting to the other instead of from both sides inwardly. The body is cast in increments which solidify in the order of placement so that the two metals are forced to retain their relative positions as placed. 70

In the continued operation of assembling the two metals, the slag is removed from the space between the bowl rings by displacement by the steel, flowing over the upper ring when rotation thereof provides the necessary force and otherwise flowing over the lower ring only and downwardly through the openings in the depressed cup section of the bowl. 75

Removal of the metal from the bowl is effected by removing the clips from the upper edge of the bowl also the upper ring after which the ring of metal is readily lifted upward. The metal thus removed is then subjected to the usual metal working operations. If the ring is desired in sections, suitable dividers may be placed at intervals between the rings in the bowl. 80

The relative sizes of the nozzles 117 and 118 100 regulates the relative rates of flow of the metals and their accompanying cooling medium and the accompanying rates of pouring where continuous flow of metal is desired. The cooling medium for each metal must be 105 of a composition that does not cause deleterious effects when entrained in the composite metal accumulation and may be powdered as well as fluid.

In Fig. 5 is shown a partial plan view of 110 the bowl 17 showing the rim and cup only. Radial arrows 120 show the direction of approach by metal and slag particles to the rim 20, while circumferential arrows 121 show the direction of rotation of the rim 20 and cup 19. It is obvious that as the particle of metal or slag in its radial movement contacts with the circumferential rotating rim 20 a spreading action occurs in the direction of the circumferential movement of the rim causing 115 a much greater attenuation of the arriving particle than would occur under impact alone. The angular movement of the wall 20 relative to the direction of approach of the metal and slag as they impact on the wall with a plastic condition of the metal is particularly effective in its operation. 120

In Fig. 6 is shown a vertical wall section of 125 the bowl arrangement of Fig. 4. Between the lower ring 108 and the upper ring 109 130

and along the wall 20 of the bowl 17 a thin inner refractory lining 122 is positioned to give protection to the vessel when extremely high temperature material is to be encountered. Due to the up and down movement of the deflector 34 or of the special distributor 112, metal is deposited in a series of folds 123, 124, which tends to result in a laminated structure of the resulting body of metal. It is obvious that the number of folds is dependent upon the rate of the up and down movement of the distributor and upon the rate of flow of metal. The successive folds of metal weld together as they form so that a solid mass of metal results when the temperature during casting permits and such procedure is preferable.

In Fig. 7 is shown the anvil 33 and deflector 34 with an accumulation of particles of metal 125 thereon cast and welded together. A small flow of metal and slag initially permits the formation of a ring nucleus to which successive particles of metal weld as they arrive and from which excess slag is projected by the rotation of the mass and by gravity. The ring stretches over the anvil under the impact of arriving metal and slag until its strength increased by cooling on the deflector is able to resist the further impacting action after which accumulation takes place in the upwardly direction. Upon removal from the anvil 33 the mass of metal may be worked into commercial bars or shapes while retaining some of the heat of casting. Speed of rotation of the anvil during the forming operation is governed to accord with the condition of the growing accumulation, being slow at the start, accelerated later, and varied from time to time as required to retain the metal in the ring.

In Fig. 8 is shown a sectional view of a pair of driven rolls 126 and 127 with water cooled passages 128 and 129 respectively. Between the rolls, and guided by roll grooves 130 and 131 respectively, thin metal strips 132 and 133 pass as the rolls revolve while slag 134 and metal particles 135 gather therebetween, the metal particles and the strips welding together and the slag departing under the roll pressure incident to the roll rotation. The continued supply of metal and slag in relative volumes of one to two and one-half respectively and at temperatures that permit the ready crystallization of the metal and its welding together under pressure forms the basis for a successful continuous casting operation in the handling of steel. Other metals may be handled in a similar manner with the slag and operating temperatures being chosen and maintained to accord with the casting characteristics of the particular metal being cast. A complete operating mechanism employing the roll equipment just described will be described and illustrated later.

In Fig. 9 is shown a simplified apparatus

for metal casting, comprising a ladle 140 with a bottom opening 141 shown in a closed condition. Into the ladle 140 slag 142 of welding cinder characteristics is introduced to serve as a heating medium for layers of cast metal 143 therein superposed on one another. Poised above the ladle 140 is shown a plunger or pressure means 144 operated by means not shown and operative to press the successive layers of cast metal 143 together and to complete their welding together while forcing the slag 142 from between the metal particles. The successive layers of cast metal may be cast and pressed exteriorly of the ladle and then be introduced into the ladle or they may be cast in the ladle individually, each being pressed out forcing the slag from between the layers and metal particles layer by layer to complete the welding into a solid mass. Successive layers of metal may be welded together sufficient to form a mass the equivalent of the usual commercial steel ingot. The mass because of its manner of assembly, particle by particle in a welding operation instead of solidification from a large molten mass, is free from the waste and defects ordinarily encountered such as piping, blowholes and segregation. The slag content is controlled by the thickness of layers cast and the pressures applied in their welding, the small masses of metal being operated on at any one time facilitating the control operations. Drainage of slag from the ladle is effected as required from time to time through opening 141 in the bottom from which a clay plug may be removed by a hand bar or other means. It is obvious that the slag temperature must be below the melting point of the metal in order that the metal may be in a weldable state, otherwise a molten metal condition would be present and nullify all the provisions in hand. The volume of slag, rate of casting and casting metal temperatures must be given due consideration in the operations involved. These factors may even be controlled to the extent of incorporating practically all of the slag into the metal cast so that no appreciable surplus remains exteriorly of the metal after the operations involved are completed.

In Fig. 10 is shown a side view and in Fig. 11 a sectional view of a machine for continuously casting metal into sheets or strips for assembly after the manner just described, in connection with Fig. 9, into an ingot, or for direct further extension by the usual rolling or drawing operations. On a base plate 145 are mounted two upright end frame plates 146 and 147 which are joined across the top by two tie plates 148 and 149. Extending through suitable bearings 150 and 151 in the end plates is a drive shaft 152 carrying on one end a power connection not shown and on the other end a pinion 153 positioned to one side and intermediate of an upper gear 154 and a

lower gear 155 respectively, which it drives. The upper gear is attached to one end of one roll 157 of a pair of parallel cooperating rolls 156 and 157 extending parallel to the drive shaft and with bearings 158, 159, 160, 161 in the end frame plates. On the ends of the rolls opposite to the upper gear 154 a pair of pinions 162 and 163 give the rolls the same rate of rotation. The lower gear 155 is attached to the end of one roll of a pair of cooperating rolls parallel to and directly below the set of rolls just mentioned, and journaled in bearings 164, 165, 166, 167 in the end plates. On the ends of the rolls opposite to the lower gear 155 a pair of pinions 168 and 169 give the rolls the same rate of rotation. The bearings of the upper pinion driven roll and of the lower pinion driven roll are adjustable horizontally by means of removable plates 170, 171, 172, 173 so that the space between the two rolls of either pair may be suitably arranged. Each roll has beveled shoulder portions 174 next to which on one side is the end bearing section 175 and on the other side a cylindrical section 176. Between the cylindrical sections a grooved section 177 is positioned. Adjacent beveled shoulders of a pair of rolls form a V notch, adjacent cylindrical sections contact with each other, and adjacent grooved sections form the outline of a passage between the rolls. Each roll has a hollow central chamber 178 with end exits 179 and pipe connections 180 for supplying a cooling medium to the central chamber. Above the upper pair of rolls and supported on the end plates, a pair of concentric pouring shells 181 and 182 are arranged. A similar pair of pouring shells 183 and 184 are arranged and supported intermediate of the upper and lower pairs of rolls. The shells adjacent the rolls have depending end portions 185, 186, 187, 188 extending downwardly to the vicinity of the rolls to partially restrain any solid or plastic material from movement toward the ends of the rolls while permitting the flow of liquids endwise of the rolls when poured thereon. Each shell 181, 182, 183, 184 respectively has its depending tapering chamber portion 189, 190, 191, 192 respectively around the top of which extends an inner lip portion 193, 194, 195, 196 respectively and an outer trough portion 197, 198, 199, 200 respectively, and an outer lip portion 201, 202, 203, 204 respectively somewhat higher than the inner lip portion. Also at one end of each shell 182, 183, 184, 185 a feed trough 205, 206, 207, 208 respectively and a guide wall 209, 210, 211, 212 respectively with a hole therethrough 213, 214, 215, 216 respectively provides a guide for the flow of liquids into the trough portions 205, 206, 207, 208 respectively from which it flows down the inclined depending shell portion onto the rolls. Below the lower pair of rolls and extending angularly downward and to the exit side of

the machine between the end plates 146 and 147 and attached thereto is positioned an apron 217 on which liquid material drops from the rolls with the solid material passing from between the rolls. Due to the roll action, solid material from between the rolls is pressed against the apron 217 and over a trough 218 to suitable receiving means in accordance with the further working which it is to receive. The liquid flows down the apron 217 to a trough 218 extending downwardly and inclined to one end of the machine draining into a ladle 219 for removal to a furnace for further use.

The concentric pouring shells are open at the tops and afford a direct passage to the rolls so that access to the rolls is always available for employment of hand tools upon the material upon the rolls, for pouring hot metal directly to the rolls from a ladle, or for the introduction of strip material to be coated between the rolls.

In the operation of the embodiment shown in Fig. 10 and Fig. 11, for casting steel, a thin temporary cross strip is placed in a folded position between each pair of rolls so as to form a dam therebetween and to feed between the rolls when they rotate. The position and action of the strip is illustrated by Fig. 8 where the ends 132 and 133 may be regarded as those of the folded strip. After warming the operating parts of the machine by pouring molten slag at a welding temperature of steel into the various shells, the operation of the casting is started by pouring welding cinder at welding heat over the upper shells of each pair of rolls while molten steel is poured from the shell 182 above and adjacent to the upper pair of rolls resulting in the formation of a pasty mass of weldable steel covered with slag on the so-called dam. The rolls 156 and 157 are then rotated at a rate in harmony with the rate of formation of the pasty mass of steel so that the dam passes between the rolls as the first end of a strip of welded and squeezed metal, rotation of the rolls serving to reduce the thickness of the metal mass, squeezing out the excess welding cinder and welding the metal particles into a coherent body. While the metal passes between the rolls 156 and 157 the molten welding cinder passes longitudinally of the rolls 156 and 157 and then downward inside the lower shell 184 and onto the second pair of rolls 174 and 175 from whence it flows onto the apron and the trough 218 and then into the ladle 219. As the lower end of the newly formed strip of metal passes between the lower pair of rolls while additions are being made to the upper end of the strip, a pasty mass of metal is formed on both sides of the product of the upper rolls while the lower pair of rolls 174 and 175 reduces the size of the pasty metal mass, squeezing out the excess welding cinder and welding the particles into a coherent

mass, so that as the strip passes out below the lower pair of rolls it is a coherent solid body of metal with a minimum of slag or welding cinder inclusions. The space between the lower pair of rolls 174 and 175 is sufficiently greater than the space between the upper pair of rolls 156 and 157 to accommodate the addition to the strip from the upper rolls of appreciable quantities of metal by the casting and welding operation just described.

As the strip continues to grow, its forward end is passed over the apron 217 and the trough 218 of the machine for further manipulation in accord with the operating plan chosen. One plan of operation contemplates folding and welding the folds together in a slag or welding cinder heating medium, as illustrated in Fig. 9 and described in connection therewith. Another plan of operation contemplates the prompt reduction by working while still retaining some of its heat of casting.

The shape of the strip produced by this embodiment is controlled by the shape of the rolls. Instead of a single flat strip resulting from the operation, a plurality of near cylindrical strips may be produced by employing suitably grooved rolls. Referring to Fig. 12, in a plan view is shown a pair of grooved rolls 220 and 221 in contact with each other along cylindrical portions 222 and 223 from the cylindrical portions of which extend beveled sections 224 and 225 to cylindrical bearing sections 226 and 227 respectively. Between the contacting cylindrical portions 222 and 223 of the pair of rolls are grooved sections 228 and 229 with edges 230 and 231 which by their adjacent positioning and cooperative action squeeze plastic material when placed thereon by their rotary movement into cylindrical sections which pass downwardly through the circular passages formed by the adjacent grooves. The adjacent cylindrical sections 222 and 223 form a trough over which liquid matter accompanying and expressed from the plastic material flows to the V or notch section formed by adjacent bevel sections 224 and 225 of the rolls. The liquid flowing away serves to convey heat from the plastic material and to cool the rolls which may be internally cooled by a separate medium as previously described.

The advantages of my invention result from reducing a cast metal from a fluid to a plastic state during the placement of the metal in its cast position. By destroying its liquid character, its ability to migrate from position to position in the casting during its cooling is destroyed. The phenomena that ordinarily manifest themselves during the change from the liquid to the solid metallic state are nullified. It is characteristic of the invention that from a liquid metal a plastic nucleus is formed to which particles of like metal are united progressively or to which

particles of a number of different metals are united. When a number of metals are so united it is contemplated that a portion of the combined metals taken from any one position shall have the same percentages of the metals as would be present in any other portion, in the case of the copper and steel previously referred to, the copper 85 per cent and steel 15 per cent. The copper acts as a matrix enclosing the steel and the uniformity of the combination is obtained by the positioning of 85 units of plastic copper and 15 units of steel regularly during the casting operation, migration of the different units being forestalled by their prereduction from molten to plastic condition.

In setting forth the steps for securing the plastic conditions of the cast metals, continued reference has been made to the use of slags of suitable characteristics. These are chosen because of their indifference to the metals. Silica combines readily with protoxide of iron and forms easily fusible silicates with which two pieces of iron at a welding heat may be coated and yet weld soundly together under pressure, the interposed liquid silicate being expelled in a greater or less degree leaving clean bright metallic surfaces of the metal to come in contact under pressure. The tribasic silicate of protoxide of iron has no action on metallic iron at high temperatures and would indeed protect the surface from oxidation and keep it bright. A silicate of this kind which is termed a "welding cinder" is desirable for the reduction of ferrous mixtures to the plastic state. Each metal has a suitable welding cinder for use in connection with the practice of this invention. However, the practice of this invention is not limited to the employment of slags, either molten or powdered, as means for obtaining the plastic and subsequently welded states. Metals, either molten or powdered, of relatively lower melting point than the metal regarded as the casting metal may be employed. Copper may be used for casting steel, in which case the copper is within the welding range of temperature of the steel. As it becomes welded in the copper, an alloy of steel and copper is formed which it is desirable to keep below 3% of copper and above 97% steel, as high percentages of copper with the steel present physical characteristics not desirable. Also in the steel matrix pure copper is held in percentages depending upon the masses and pressures used during the welding operations. This is in contrast to the previously mentioned combination of copper 85 per cent and steel 15 per cent where the copper serves as a matrix holding the steel in definite placement.

While suitable slags are indifferent to the metals being cast, the metalloids in the mixtures with the metals are sometimes attacked to the detriment of the final product unless

due precautions are employed. Such precautions involve the provision of an excess of the metalloids beyond the requirements of the final product in the solid condition particularly when washing by slag is practiced.

5 When slag approximately in an amount to be incorporated in the cast metal and in either powdered or molten condition or of a regulated specific gravity is chosen, such precautions referred to are not so essential. 10 Whether these metalloids are in the metal prior to the casting process or whether they are added during the process of casting is immaterial. The use of a slag to cover a 15 metal, which is to reduce another metal to a plastic state is contemplated. Thus, copper into which steel may be cast may be covered with slag which may serve the dual purpose of protecting the copper and reducing the 20 alloying action between the copper and steel.

Many changes may be made in the apparatus employed, as well as in the steps of my process, without departing from my invention. Within the scope of my claims, parts 25 of my complete process forming sub-processes may be used, without departing from my invention. The materials used, the pressure apparatus and the receiving apparatus 30 may be widely varied.

I claim:

1. In the process of casting metal, the steps consisting of entraining welding slag particles in a body of molten metal thereby 35 reducing the metal to welding temperature, welding the metal into a solid body and expressing excess slag particles while continuing said entraining operation.

2. In the process of casting steel, the steps 40 consisting of entraining welding slag particles in a body of molten steel thereby reducing the said steel to welding temperature, expressing excess slag particles and welding the metal into a solid body while continuing 45 said entraining operation.

3. The method of casting metal comprising the steps of entraining slag particles in a body of molten metal thereby reducing the metal to welding temperature, welding the 50 body of metal upon itself and expressing excess slag particles.

4. The method of casting metal, consisting 55 in changing the molten metal into a coherent mass by contact with cooling means comprising metal or slag or both so obtaining the welding temperature range of the metal being cast, expressing entrained portions of the liquid cooling means from said coherent mass and welding the metal where 60 perforated by said expressed entrained portions.

5. The method of casting metal, consisting 65 in changing the molten metal into a coherent mass by contact with liquid cooling means comprising either metal or slag with-

in the welding temperature range of the metal being cast, expressing entrained portions of the liquid cooling means from said coherent mass and adding progressively metal to said coherent mass.

6. In the process of casting metal, the steps 70 consisting of entraining material particles in a body of molten metal thereby reducing the metal to welding temperature, expressing excess material particles while continuing said entraining operation, and welding the metal into a solid body.

7. In the process of casting steel, the steps 75 consisting of changing the molten metal into a weldable condition while retaining some of the heat of casting, welding metal particles together under the protection of a welding slag, expressing entrained portion of said slag, and progressively casting additional particles on the welded mass.

8. The method of casting metal, consisting 80 in adding additional metalloids to the molten metal, changing the molten metal into a coherent mass by contact with cooling means comprising metal or slag or both so that a mean temperature within the welding range of the cast metal results, and expressing entrained portions of the cooling means from said coherent mass.

9. In the process of casting a ferrous metal 85 compound, the step consisting of adding a protective metalloid to the molten metal to be cast, then forcing a slag of puddling characteristics therethrough while the metal is being cast.

10. In the process of casting steel, the step 90 consisting of adding a protective metalloid to the molten steel to be cast, then forcing a slag of puddling characteristics therethrough while the metal is being cast, where- 105 by the metal is cooled.

11. The method of casting a plurality of metals into a single mass comprising the steps of reducing each metal from a molten to a welding condition, welding said metals together in small particles, and repeatedly adding small particles in regular alternation of metals by welding while retaining heat from the original casting.

12. In the process of casting an alloy steel, 110 the step consisting of adding a protective metalloid to the alloy steel to be cast, then forcing a slag of puddling characteristics therethrough while the metal is being cast, whereby the metal is cooled.

13. In the process of casting steel into an alloy the step consisting of adding a protective metalloid to the molten steel, simultaneously casting the molten steel into contact with an alloying metal and forcing a slag 125 of puddling characteristics therethrough.

14. In the process of casting metal, the step 130 consisting of forcing a slag of puddling characteristics therethrough while the metal is being cast and regulating the temperature of

the slag within the welding range of the metal.

15. In the process of casting ferrous metal, the step consisting of forcing a slag of puddling characteristics through the metal while the metal is being cast, regulating the temperature of the slag within the welding range of the metal and welding the metal.

16. As an article of manufacture, a composite metal body comprising a plurality of metal particles having an individual analysis, between said particles a plurality of metal particles having another individual analysis, said particles being welded along their faces of contact from a plastic state while preserving within their lines of contact each its individual analysis.

17. As an article of manufacture, a composite metal body comprising a plurality of steel particles having the same analysis, between said particles a plurality of metal particles of another analysis, and a weld between adjacent particles so positioned effective to hold them as a body.

18. As an article of manufacture, a composite metal body comprising a plurality of steel particles having the same analysis, between said particles a plurality of particles of steel having another analysis, and a weld between adjacent particles so positioned effective to hold them as a body.

19. A casting machine comprising a molten metal supply means, a molten slag supply means, means for contacting said slag on said metal whereby the temperature of said metal is reduced to a welding range, and welding means effective to weld together said metal in the welding temperature range.

In testimony whereof I affix my signature.  
MARTIN E. EVANS.

46

45

50

55

60

65